# EUROPEAN PATENT SPECIFICATION

(11) **EP 1 274 895 B1**
(45) Date of publication and mention of the grant of the patent: **27.04.2005**
(21) Application number: 01913056.6
(22) Date of filing: 26.02.2001
(51) Int. Cl.: D06P 1/00, D06P 3/82, D06B 11/00

(54) **MULTICOLOR FLOORING ARTICLE**
MEHRFARBIGER FUSSBODENBELAG
ARTICLE DE REVETEMENT POUR SOL MULTICOLORE

(30) Priority: 24.03.2000 US 535442
(43) Date of publication of application: 15.01.2003
(73) Proprietor: INVISTA Technologies S.à.r.l., Wilmington, DE 19808 (US)
(72) Inventor: TUNG, Wae-Hai, Marietta, GA 30062 (US)
(74) Representative: Carpmaels & Ransford
(86) International application number: PCT/US2001/006097
(87) International publication number: WO 2001/073189

(56) References cited:
- US-A- 3 101 522
- US-A- 3 439 999
- US-A- 5 160 347
- US-A- 5 199 958

## Description

### FIELD OF THE INVENTION

The invention relates to a multicolor flooring article, and more particularly a multicolor carpet made from a combined yarn comprising at least three component synthetic yarns.

### BACKGROUND OF THE INVENTION

Multicolor flooring articles, such as carpets, are desired by designers and consumers to add diversity and flexibility to the aesthetics of carpets over solid color carpet. One conventional method of making a multicolor carpet is to make it from yarns which are themselves combinations of component yarns having different dyeabilities and then to dye the carpet using a mixture of dyes such as acid and cationic. For example, nylon yarns with deep acid, light acid and cationic dyeabilities may be combined by twisting them together or commingling them with high pressure air forming a combined yarn. The combined yarn may be tufted or woven to form a carpet, and the carpet may then be dyed in a dye bath containing acid and cationic dyestuffs. In this example, since two of the three yarn components are acid dyeable, the combined yarn will always include two component yarns dyed in the same color family, having light and deep shades of the same color. Thus, it is not possible to dye this combined yarn in such a way that it has three entirely different colors, i.e. the color styling flexibility of the carpet is limited.

Another process for making multicolor carpets is to combine acid and cationic dyeable nylon yarns with a polyethylene terephthalate (abbreviated PET or alternately, 2GT). PET is inert to acid and cationic dyes and can only be dyed with disperse dyes. PET (unmodified) is not suitable for dyeing on a continuous dye line, or equipment designed to dye carpet on a continuous basis, because the dye leveling or uniformity of the dye is poor. Dyeing on a continuous dye line is the most economical method for dyeing carpet. Poor dye leveling occurs when the fiber has low dyeability in terms of dye rate and dye exhaust that results in poor dye uniformity and splotchiness. PET can be dyed with disperse dyes in conjunction with a carrier. A carrier is an organic chemical used to swell or open the polymer structure of the PET fiber so that the fiber may be dyed acceptably in a high speed continuous dyeing process. However, carriers are costly and toxic. A carpet using this combination of yarns when dyed with acid, cationic and disperse dyestuffs and carrier can result in a multicolor effect in which each color of a yarn component is different from the other. However, these carpets have poor resistance to crushing and matting, due to the poor resiliency of the PET yarn component. Thus, the multicolor carpet made in this manner is not a desirable option because the crushing resistance is unacceptable and requires a costly and toxic carrier.

The following disclosures may be relevant to various aspects of the present invention and may be briefly summarized as follows:

U.S. Pat. No. 5, 160, 347 to Kay et al. discloses carrier dyeable polyester yarns that are space dyed by spraying with water dispersions of disperse dyes without thickeners or carriers followed by a short steaming process and autoclaving to develop the dyes or by a process of knitting the yarn into socks or tubes which are roller printed with disperse dyestuff, thickener and carrier dissolved in water in various colors followed by steaming, washing, drying and deknitting. The thus produced space dyed yarns are then tufted into area rugs along with undyed yarns of "carrierless" polyester fibers and/or nylon fibers and dyed with a cationic, acid or disperse dye appropriate to the dye receptivity of the undyed yarns while avoiding overdyeing of the space dyed yarns to produce a multi-color piece dyed area rug.

U.S. Pat. No. 5, 354, 342 to Jenkins discloses stain-resistant, multicolored cationic dyeable carpet fibers space dyed with an acid dye or premetalized acid dye, heatset, then tufted together with undyed cationic dyeable nylon fibers into a carpet. The carpet is then overdyed with an acid dye or premetalized acid dye to selectively dye only the previously undyed cationic dyeable nylon fibers, without staining or discoloring the adjacent previously dyed fibers, resulting in a multicolored stain resistant carpet.

U.S.Pat. No. 5, 199, 958 to Jenkins et al. discloses a multicolored stain-resistant nylon carpet prepared by tufting a space dyed cationic-dyeable carpet nylon, dyed with an acid or premetalized dye intermixed and tufted with an acid dyeable nylon and overdyed with an acid dye to selectively dye the acid dyeable fibers but not the already space dyed yarns.

U.S. Pat. No. 3, 652,198 to Farber et al. discloses a process for dyeing fibers, fabrics or other shaped articles made from blends of either poly (alphaolefins) or polyesters and various thermoplastic nitrogen-containing basic polymers to a multicolor pattern.

It is desirable to have a system for dyeing a multicomponent carpet in which each of component of three component yarns may be dyed a different color without the use of a carrier and the resultant carpet has a high resistance to crushing and matting.

### SUMMARY OF THE INVENTION

Briefly stated, and in accordance with one aspect of the present invention, there is provided a multicolor flooring article comprising combined yarns, each combined yarn comprising at least an acid dyeable nylon multifilament yarn, at least a cationically dyeable nylon multifilament yarn and at least a poly(trimethylene terephthalate) multifilament yarn wherein the flooring article is dyed at least three different colors in a carrier free dye bath containing a combination of acid dye, cationic dye and disperse dye.

Pursuant to another aspect of the present invention, there is provided a process for making a multicolor flooring article comprising the steps of: combining at least an acid dyeable nylon multifilament yarn, at least a cationically dyeable nylon multifilament yarn and at least a poly(trimethylene terephthalate) multifilament yarn forming a combined yarn; making a flooring article using the combined yarn; and dyeing the flooring article at least three different colors in a carrier free dye bath using acid dyes, cationic dyes and carrier-free disperse dyes.

### BRIEF DESCRIPTION OF THE DRAWINGS

Other features of the present invention will become apparent as the following description proceeds and upon reference to the drawing, in which:
Figure 1 is a schematic illustration of an embodiment of the present invention of a combined yarn comprising three component yarns twisted together.

While the present invention will be described in connection with a preferred embodiment thereof, it will be understood that it is not intended to limit the invention to that embodiment. On the contrary, it is intended to cover all alternatives, modifications, and equivalents as may be included within the scope of the invention as defined by the appended claims.

### DETAILED DESCRIPTION OF THE INVENTION

The present invention provides versatility in multicolored flooring articles such as rugs and carpets. In an embodiment of the present invention, the combined yarn comprises at least two polyamide yarns and at least one poly(trimethylene terephthalate) (i.e. PTT) yarn for at least three distinct colors for the flooring article. The two polyamide yarns useful for an embodiment of the present invention include any known bulked continuous filament (i.e. BCF) or yarn of either type nylon 6 or nylon 6,6 polymer. Such yarns are commonly used in carpet manufacturing. The linear density, or denier, of these yarns typically range between about 500 and about 2800. In an embodiment of the present invention, at least one of the polyamide yarns is dyeable by acid dyestuffs. The dyeability of these yarns can vary from light, to medium to deep in color. Additionally, at least another of the polyamide yarns useful for the invention is dyeable by cationic dyestuffs. Thirdly, at least one poly(trimethylene terephthalate) yarn useful for the invention is any known bulked continuous filament yarn. The denier of this yarn also ranges between about 500 and about 2800.

The polyamide and PTT multifilament yarns, of an embodiment of the present invention, are combined by either air entangling or cable twisting together. Several methods of air entangling (for example, those described in US Patent 3,978,558 ) and cable twisting (for example, the one described in US Patent 3, 368,336 ) are well known in the art. Any of the known methods may be applied in the present invention. Combining the yarns by air entangling results in a yarn having colors that are blended and generally muted. Combining the yarns by cable twisting results in a yarn having more color separation. Typically, three yarns of 500 to 2800 denier* each are combined by either method.
* 1 denier = 0.9 d Tex

Referring now to the drawings, where the showing is for the purpose of describing a preferred embodiment of the invention and not for limiting same. For clarity the Figure is drawn outside of scale. Figure 1 illustrates a cable twisted combined yarn 10 where yarn 1 is an acid dyeable polyamide yarn, yarn 2 is a cationically dyeable polyamide yarn and yarn 3 is a poly(trimethylene terephthalate) yarn. Additional yarns may also be included in the combined yarn to give a desired aesthetic in the resulting carpet.

The multicolor carpet according to an embodiment of the present invention is made by tufting or weaving in a conventional manner, preferably by tufting. A typical carpet construction of the present invention is about 0.04 to about 0.27 g/cm² (12 to about 80 oz. weight per square yard) with 0.3175 to 2.54 cm (1/8" to 1") pile height. The multicolor carpet is preferably loop pile, although it may also be cut pile. Loop pile provides a better view of the different colors in the carpet.

The carpet is dyed with a combination of acid, cationic and disperse dyes in a bath that is carrier-free. By "carrier-free" is meant that no carrier is present in the dyeing process. Each yarn (yarns 1, 2 and 3 from Figure 1) when dyed is receptive to different dyes. For example, yarn 1 being acid dyeable, has its color determined by the acid dye and disperse dye; yarn 2 being cationically dyeable, is more receptive to the cationic dye and disperse dye; and yarn 3's color determination is determined by the carrier free disperse dye only. Thus, providing at least three distinct colors for an aesthetically pleasing multi-color carpet.

The carpet may be dyed using a conventional dyeing process, such as that used with continuous range dyers such as a commercially available dyeing unit from Kuster Corporation. In continuous range dyeing, first the dyestuffs are sprayed onto the carpet. The dyes are applied in amounts ranging from about 0.01% to about 2%, but preferably between about 0.01% to about 1%, of the weight of the fiber. The carpet is then steamed for about 2 to about 5 minutes at temperatures typically about 210 to about 212 degrees F. The carpet is then rinsed and dried. While the continuous dye line process is preferred, the present invention is applicable to a batch process (such as Beck dyeing).

The dyed carpet of the present invention has excellent pile height retention. The carpet of the present invention has a pile height retention of at least 85% and preferably at least 90%, when subjected to the Vetterman Drum Test.

### Test Method

### Vetterman Drum Test

The test carpet samples are cut into 26.67 cm x 26.67 cm (10.5" x 10.5") size and conditioned in a constant temperature (70 F) and humidity (65% RH) room for 24 hours. The samples are then placed into a Vetterman drum and secured by a retaining ring. The samples are subjected to a 5,000 cycles test (ASTM D5417-93). The tested samples are then conditioned in a constant temperature (70 F) and humidity (65% RH) room for 24 hours. The pile heights of tested samples are then measured by inserting a ruler into the pile of a carpet and then reading the height of the pile in inches. (The thickness of the backing and latex coating are excluded.)

The pile height retention is calculated as follows:$\text{pile height retention =} \frac{\text{pile height after 5,000 cycles}}{\text{pile height before test}} \text{x100%}$

An embodiment of the present invention is illustrated by the following example:

### Example

A combined yarn was formed by commingling on a Belmont intermingling machine (available from Belmont Textile Machinery Company, Belmont, NC) the following component yarns: one 2400 denier acid dyeable nylon BCF yarn, one 2400 cationically dyeable nylon BCF yarn and four 1100 denier poly(trimethylene terephthalate) BCF yarns. A control combined yarn was formed by commingling the same yarns, substituting four 1100 denier poly(ethylene terephthalate) BCF yarns for the four poly(trimethylene terephthalate) yarns.

The example and control yarns were tufted into 907.2 g (32 ounce) loop pile carpets on a 5/32 inch gauge (1 inch=25.4 mm) tufting) machine. The carpets were then dyed on a continuous Kuster range dyer (available from the Zima Corporation, Spartanburg, South Carolina). The dyestuffs were sprayed onto the carpet before steaming for dye fixation. The following dye formulations and conditions were used:
acid dyes Tectilon (available from Ciba-Geigy AG, Basel Switzerland)

| | |
|---|---|
| orange 3G | 0.075% |
| red 2B | 0.075% |
| blue 4R | 0.075% |

cationic dyes Sevron (available from Crompton & Knowles Colors Incorporated, Charlotte, NC)

| | |
|---|---|
| yellow 3RL | 0.0025% |
| red YCN | 0.0063% |
| blue AN | 0.0188% |

disperse dyes Intrasil (available from Crompton & Knowles Colors Incorporated)

| | |
|---|---|
| red QE | 0.05% |

The dye liquor was applied at 450 to 500% wet pick up. The pH of the dye liquor was adjusted to 6-6.5. The dwell time in the steam was 3.8 minutes.

The resulting carpets included attractive three color aesthetics. The carpets were subjected to the Vetterman Drum Test for 5,000 cycles. The samples were conditioned in a 70 degree F, 65% relative humidity room for 24 hours. The pile height was measured for each carpet before and after the test. The percent recovery of each carpet was calculated from the pile height measurements using the above formula.

| | pile height (inches*) | | pile height retention (%) |
|---|---|---|---|
| | before test | after test | |
| Example | 0.344 | 0.313 | 91 |
| Control | 0.375 | 0.189 | 50 |

| | | | |
|---|---|---|---|
| * inch = 25.4 mm. | | | |

## Claims

1. A multicolor flooring article comprising combined yarns, each of the combined yarns comprising at least an acid dyeable nylon multifilament yarn, at least a cationically dyeable nylon multifilament yarn and at least a poly(trimethylene terephthalate) multifilament yarn wherein the flooring article is dyed at least three different colors in a carrier-free bath containing a combination of acid dye, cationic dye and disperse dye.

2. The multicolor flooring article of claim 1, comprising a pile height retention of at least 85% when subjected to the Vetterman Drum Test.

3. The multicolor flooring article of claim 2, comprising a pile height retention of at least 90% when subjected to the Vetterman Drum Test.

4. The multicolor flooring article of claim 1, wherein the combined yarns are combined by cable twisting.

5. The multicolor flooring article of claim 1, wherein the combined yarns are combined by commingling with high pressure air.

6. The multicolor flooring article of claim 1, wherein each yarn of the combined yarns is dyed one of at least three different colors and differ in color from two of the other multifilament yarns of the combined yarn.

7. The multicolor flooring article of claim 1, comprises a carpet.

8. A process for making a multicolor flooring article comprising the steps of:
a. combining at least an acid dyeable nylon multifilament yarn, at least a cationically dyeable nylon multifilament yarn and at least a poly(trimethylene terephthalate) multifilament yarn forming a combined yarn;
b. making a flooring article using the combined yarn; and
c. dyeing the flooring article at least three different colors in a carrier free dye bath using acid dyes, cationic dyes and disperse dyes.

9. The process of claims 8, wherein the combining step comprises cable twisting or commingling with high pressure air.

10. The process of claim 8, wherein each multifilament yarn of the combined yarn is dyed one of the three different colors and differ in color from two of the other multifilament yarns of the combined yarn.

11. The process of claim 8, wherein the making step comprises tufting or weaving.

12. The process of claim 8, wherein the multicolor flooring article comprises a carpet.

## Patentansprüche

1. Mehrfarbiger Fußbodenbelag, aufweisend kombinierte Garne, wobei jedes der kombinierten Garne mindestens ein säurefärbbares Multifilament-Nylongarn aufweist, mindestens ein kationisch färbbares Multifilament-Nylongarn und mindestens ein Multifilament-Poly(trimethylenterephthalat)-Garn, wobei der Fußbodenbelag mit mindestens 3 verschiedenen Farben in einem carrierfreien Bad gefärbt ist, das eine Kombination von saurem Farbstoff, kationischem Farbstoff und Dispersionsfarbstoff enthält.

2. Mehrfarbiger Fußbodenbelag nach Anspruch 1, aufweisend eine Florhöhen-Retention von mindestens 85%, wenn er dem Trommeltest nach Vetterman unterworfen wird.

3. Mehrfarbiger Fußbodenbelag nach Anspruch 2, aufweisend eine Florhöhen-Retention von mindestens 90%, wenn er dem Trommeltest nach Vetterman unterworfen wird.

4. Mehrfarbiger Fußbodenbelag nach Anspruch 1, wobei die kombinierten Garne mit Hilfe eines Verzwirnens vereint werden.

5. Mehrfarbiger Fußbodenbelag nach Anspruch 1, wobei die kombinierten Game durch Verwirbeln mit hohem Luftdruck vereint werden.

6. Mehrfarbiger Fußbodenbelag nach Anspruch 1, wobei jedes Garn der kombinierten Game mit mindestens einer von drei verschiedenen Farben gefärbt ist und sich in der Farbe von zwei der anderen Multifilamentgarne des kombinierten Garns unterscheidet.

7. Mehrfarbiger Fußbodenbelag nach Anspruch 1, umfassend einen Teppich.

8. Verfahren zum Herstellen eines mehrfarbigen Fußbodenbelags, umfassend die Schritte:
a. Kombinieren von mindestens einem säurefärbbaren Nylon-Multifilamentgarn, mindestens einem kationisch färbbaren Nylon-Multifilamentgarn und mindestens einem Poly(trimethylenterephthalat)-Multifilamentgarn unter Erzeugung eines kombinierten Garns;
b. Herstellen eines Fußbodenbelags unter Verwendung des kombinierten Garns; und
c. Färben des Fußbodenbelags mit mindestens drei verschiedenen Farben in einem carrierfreien Farbstoffbad unter Verwendung von sauren Farbstoffen, kationischen Farbstoffen und Dispersionsfarbstoffen.

9. Verfahren nach Anspruch 8, bei welchem der Schritt des Kombinierens ein Verzwirnen oder Verwirbeln mit hohem Luftdruck umfasst.

10. Verfahren nach Anspruch 8, bei welchem jedes der Multifilamentgarne des kombinierten Garns mit einer von den drei verschiedenen Farben gefärbt ist und sich in der Farbe von zwei der anderen Multifilamentgarne des kombinierten Garns unterscheidet.

11. Verfahren nach Anspruch 8, worin der Herstellungsschritt ein Tuften oder Weben umfasst.

12. Verfahren nach Anspruch 8, bei welchem der mehrfarbige Fußbodenbelag einen Teppich umfasst.

## Revendications

1. Article de revêtement pour sol multicolore comprenant des fils combinés, chacun des fils combinés comprenant au moins un fil multifilament de nylon apte à la coloration acide, au moins un fil multifilament de nylon apte à la coloration cationique et au moins un fil multifilament de poly(triméthylène téréphtalate) dans lequel l'article de revêtement pour sol est coloré d'au moins trois couleurs différentes dans un bain exempt de support contenant une combinaison de colorant acide, de colorant cationique et de colorant dispersé.

2. Article de revêtement pour sol multicolore de la revendication 1, comprenant une rétention de hauteur de pile d'au moins 85% lorsqu'il est soumis au test du tambour de Vetterman.

3. Article de revêtement pour sol multicolore de la revendication 2, comprenant une rétention de hauteur de pile d'au moins 90% lorsqu'il est soumis au test du tambour de Vetterman.

4. Article de revêtement pour sol multicolore de la revendication 1, dans lequel la combinaison des fils combinés est réalisée par torsion de câble.

5. Article de revêtement pour sol multicolore de la revendication 1, dans lequel la combinaison des fils combinés est réalisée par co-mélange avec de l'air sous haute pression.

6. Article de revêtement pour sol multicolore de la revendication 1, dans lequel chaque fil des fils combinés est coloré d'une couleur parmi au moins trois couleurs différentes et diffère en couleur de deux des autres fils multifilaments du fil combiné.

7. Article de revêtement pour sol multicolore de la revendication 1, constitué d'un tapis.

8. Procédé de fabrication d'un article de revêtement pour sol multicolore comprenant les étapes consistant à:
a. combiner au moins un fil multifilament de nylon apte à la coloration acide, au moins un fil multifilament de nylon apte à la coloration cationique et au moins un fil multifilament de poly(triméthylène téréphtalate) de manière à former un fil combiné;
b. fabriquer un article de revêtement pour sol en utilisant le fil combiné; et
c. colorer l'article de revêtement pour sol d'au moins trois couleurs différentes dans un bain de colorant exempt de support utilisant des colorants acides, des colorants cationiques et des colorants dispersés.

9. Procédé de la revendication 8, dans lequel l'étape de combinaison comprend la torsion de câble ou le co-mélange avec de l'air sous haute pression.

10. Procédé de la revendication 8, dans lequel chaque fil multifilament du fil combiné est coloré d'une couleur parmi les trois couleurs différentes et diffère en couleur de deux des autres fils multifilaments du fil combiné.

11. Procédé de la revendication 8, dans lequel l'étape de fabrication est constituée de touffetage ou de tissage.

12. Procédé de la revendication 8, dans lequel l'article de revêtement pour sol multicolore est constitué d'un tapis.
